# EUROPEAN PATENT SPECIFICATION

(11) **EP 0 117 383 B1**
(45) Date of publication and mention of the grant of the patent: **26.10.1988**
(21) Application number: 83850190.6
(22) Date of filing: 06.07.1983
(51) Int. Cl.: C10C 3/02

(54) **Oxidation-resistant pitches**
Oxydationswiderstandsfähige Peche
Des brais résistants à l'oxydation

(30) Priority: 25.02.1983 CA 422361
(43) Date of publication of application: 05.09.1984
(73) Proprietor: Carbochem Inc., Mississauga, Ontario L4W 2V4 (CA)
(72) Inventor: Cukier, Samuel, Toronto Ontario M6B 3G5 (CA); Kremer, Henry A. F .L., Thornhill Ontario L4J 1Ml (CA)
(74) Representative: Nilsson, Nils Erik

(56) References cited:
- FR-A- 879 656
- US-A- 2 669 525
- US-A- 3 539 370
- US-A- 4 298 396
- CHEMICAL ABSTRACTS, vol. 89, no. 4, July 24, 1978, page 176, no. 27394f, Columbus, Ohio, US; & RO - A - 58 599 (CRETULESCU, CONSTANTIN) 30-09-1975
- Kirk-Othmer, "Encyclopedia of Chemical Technology", 3rd Edition, vol. 3, 1978, p. 284

## Description

### Field of the invention

This invention is directed to a process for making pitch compositions which are more resistant to oxidation, and preferable to those yielding more stable, less porous anodes producing less fumes and less gasification, and or to pitches used as refractory materials.

### Background of the invention

A preponderant number of applications which entail the use of coal tar or petroleum pitches require the carbonization of the pitch material. Examples of carbonization processes include coking and graphitization. During the carbonization process, it is normal to lose between 25 and 65% of the binder, the exact loss being dependent on the volatile content of the pitch. The loss of volatiles to the environment is additionally undesirable in that they constitute a source of air pollution. It is common practice in the industry to indicate this weight loss by the fraction of the starting material which remains upon carbonization, eg. the fraction of the material remaining upon coking is called the "coking value" of the pitch. This is particularly important when the pitch is used as a binder in the formation of coked carbon bodies.

Generally a carbon electrode is a two-phase or binary carbon system consisting of a petroleum coke filler (an aggregate with a specific size distribution) whose particles are bound by a pitch coke phase (called binder pitches) which is developed during carbonization of the electrode paste. In aluminum production, the carbon particles disintegrate from the working surface of an anode by selective oxidation of the binder pitch and thus form carbon dust. The binder pitch phase of anodes is consumed preferentially during oxidation, both electrolytically and chemically; this also results in dusting and the net effect is that carbon consumption is significantly more than the stoichiometric requirement sometimes doubling the stoichiometric amount. This is a substantial amount, if one considers that 83-90% of the anode is carbon filled

Also a problem encountered with baked carbon bodies obtained from pitches is their relatively high oxidation rate, particularly noticeable when they are used as refractory materials or as electrodes. This oxidation rate can be attributed to such factors as the porosity of the carbon body, its specific surface and the inorganic impurities present in the carbon body.

Techniques hitherto employed to decrease this oxidation rate include pressure impregnation or coating of previously baked carbon bodies with aqueous solutions of oxidation retardant materials such as phosphates, silicates, etc., after which the carbon bodies are rebaked to drive away the moisture. While the former technique requires pressure treating equipment and large volumes of an often expensive impregnant, neither technique succeeds in inhibiting oxidation throughout the interior of the carbon body.

British Patent 865,320 teaches adding oxidation inhibitors to the coke filler-pitch mix before baking. This technique however, requires 4 to 20% weight of the corresponding mix, of the additive. This is expensive in comparison to the base material being treated. Such large amounts of additive may have a deleterious effect if the resulting carbon body is used for making an electrode. During electrolysis such additives are normally incombustible and constitute a substantial portion of the electrode which may form residues and contaminate the system.

Also U.S. Patent No. 4,298,396, dated November 3, 1981 as invented by Limonchik et al, describes systems improving oxidation resistance of anodes in such systems however, dusting is not improved.

### Brief description of the present invention

It is therefore the object of the present invention to provide a more resistant pitch composition which has increased coking value. It is also an object of this invention to provide a pitch which upon carbonization yields a carbon body having improved oxidation resistance.

Another object of the invention is to decrease the rate of oxidation of carbon bodies and in particular of carbon electrodes used in the aluminum industry.

Still another object of the invention is to reduce the dusting.

Another object of the invention is to reduce the consumption rate of the carbon electrode that is of both the pitch coke carbon which provides the binder phase and the filler carbon, thereby achieving considerable savings.

Accordingly the invention is directed to the use of an active component comprising at least one member selected from the class consisting of alkyl-aryl sulfonic acid, and alkyl-aryl sulfonates, wherein the alkyl group of said aryl sulfonic acid or aryl sulfonate is a member selected from the class consisting of branched and unbranched alkyl members having from one to four carbon atoms and the sulfonates are salts of the metals selected from the class consisting of groups 1 and 2 of the periodic table, and ammonium, in a process for making electrodes having a good resistance to oxidation at high temperature which comprises: treating a binder or impregnating material for electrodes with an effective amount of the active component above the softening point of the pitch but at a temperature not exceeding 200°C, said member being compatible with and soluble in said pitch when in a molten state and said amount being less than 1% by weight of said pitch, and wherein the pitch when being an impregnating pitch is mixed with coke prior to melting.

By soluble in said pitch is meant that the active component must dissolve in the molten pitch.

By the expression "said member being compatible with said pitch" is meant a member which will not add atoms or molecules detrimental to anodes or to the electrolytic bath. Examples of such compatible members include: pitch-soluble alkyl-aryl sulfonates of the aromatic family, that is those containing rings such as anthracene, naphthalene, benzene of the alkyl-aryl sulfonates family such as alkyl-benzene sulfonates, alkyl-naphthalene sulfonates and alkyl-anthracene sulfonates and homologues where the cation is at least one member selected from the class consisting of metals of groups 1 and 2 of the periodic table as well as ammonium and preferably sodium, potassium, ammonium ion and the like; and the alkyl is a branched or unbranched chain having between 1 and 4 carbon atoms.

### Detailed description of the preferred embodiment

The preferred sulfonated members of the active component are the sulfonated naphthalene compounds and homologues which are preferably used in amounts of the order of ppm, for instance 200 to 5000 ppm. This amount may vary widely according to the pitch used, and the temperature and other experimental conditions, but is generally less than 1 %. The treatment must be made above the softening point of the pitch but generally below 200°C, in order to avoid premature degradation of the sulfonic acid in the sulfonate.

The treatment is generally made by mixing the softened pitch with the active component with or without other additives, such as those used in the making of electrodes or refractory materials. For instance in the making of electrodes, the treatment can be made when coke is mixed with the binding pitch: For instance, the pitch material may be a binder pitch for electrodes which is mixed with coke prior to melting.

The following examples will serve to illustrate the invention.

### Example 1

In a series of experiments sulfonated naphthalene compounds known under the trade mark "CEDEPON AT-400" TM were added in various concentrations ranging from 300 to 2000 ppm based on the total weight of the pitch, mixed in the heated liquid pitch at about 180°C. Mixing time was half an hour.

Surprisingly an increase in the softening point (as determined by the cube in air, ASTM D-2319), and an increase in coking value (as determined by the British Standard of Testing Tar and its Products PT 10-79) were found as shown in Table 1 herein below.

### Example 2

The following example is illustrative of the physical properties of the new pitch composition.

### Pitch preparation

Aluminum Grade Flaked Coal Tar Binder Pitch was melted carefully without overheating and kept at a temperature of 180°C±5°C. The sulfonated naphthalene available under the Trademark "CEDEPON", in concentrations of 1000 ppm, was added to the continuously agitated molten pitch and mixed up for 30 minutes until visual homogeneity then cooled and broken up to lumps. The physical properties of the new pitch composition at 1000 ppm were measured and compared against the physical properties of the untreated pitch compositions. Results are shown in Table 2 hereinbelow.

### Example 3

The following example is illustrative of the typical oxidation resistance of the new pitch compositions.

### Electrode preparation and testing

All experiments used "Domtar" Aluminum Grade Binder Pitches. In the first group of experiments, small electrodes were prepared with a North American commercially used petroleum coke by using various recipes. The levels of sulforated naphthalene "CEDEPON AT 400 TM" included in the mixture were varied in an industrial formula. Small electrodes (10 mm diameter) were extruded and baked.

In a different series of experiments, electrodes were produced in a Pilot Plant based on a European standard petroleum coke. The anodes were baked after moulding. Test cylinders were then cut from the various electrodes for testing, as disclosed in A. M. Odok and W. K. Fischer, "Application of Pilot Plant Work in Prebaked Anode Manufacturing", pp. 269-286 in Light Metals, Vol. 1, John J. Miller, ed.: A.I.M.E., New York, N.Y., 1978.

The electrode consumption tests were conducted in a furnace at approximately 960°C for 7 hours, passing a measured amount of carbon dioxide through the furnace. Other physical properties have been determined by standard testing methods.

It was found that applicant's novel pitch compositions were the most resistant to carbon dioxide at high temperatures in comparison with other North American binder pitches supplied to aluminum manufacturers. Tests have been carried out at various additive levels with improved results. (Table 3). At A 2000 ppm additive level, the anode residue increased by 65% and the dusting decreased by 53% at 30% Butts level in the mix.

In the second series of experiments, a different batch of Pitch was used and C0₂ reactivity tests were carried out similarly to the first series of experiments and purposely with the addition of butts. The results as shown in Table 4 indicate that the addition of 30% Butts have deteriorated the anode performance significantly (32% drop in residue and 89% increase in dusting). The usage of additive however, compensated for the losses; at 1000 ppm additive level the reactivity and dusting has returned to normal level (i.e., when no Butts had been used); at 2000 ppm additive level, the improvements were even greater and 12% increase of the residue and over 20% decrease in dusting has been achieved over the standard anode made without butts.

Determination of deleterious key elements (i.e. sulfur, phosphorus, silica, etc.) in the electrode, as is known in the prior art indicated that no increase had been detected in these elements from the sulfonated active component.

In summary the alkyl-aryl sulfonated active component has clearly demonstrated its effectiveness in improving the quality of the electrode. Significant improvements could be achieved by using the active component described above, in a recipe utilizing a less than inert petroleum coke filler. The amount of gasification and dusting has been reduced, thereby increasing the yield of aluminum production with the improved electrode. The realization of these benefits would be of great economic advantage, compensating for the ever increasing reactivity of regular petroleum cokes.

The pitches described hereinabove because of their improved physical properties may also be advantageously used as refractory materials, as is known by those skilled in the art.

Modification may be made without departing from the spirit of the invention as defined in the appended claims.

## Claims

1. The use of an active component comprising at least one member selected from the class consisting of alkyl-aryl sulfonic acid, and alkyl-aryl sulfonates, wherein the alkyl group of said aryl sulfonic acid or aryl sulfonate is a member selected from the class consisting of branched and unbranched alkyl members having from one to four carbon atoms and the sulfonates are salts of the metals selected from the class consisting of groups 1 and 2 of the periodic table, and ammonium, in a process for making electrodes having a good resistance to oxidation at high temperature which comprises: treating a binder or impregnating material for electrodes with an effective amount of the active component above the softening point of the pitch but at a temperature not exceeding 200°C, said member being compatible with and soluble in said pitch when in a molten state and said amount being less than 1% by weight of said pitch, and wherein the pitch when being an impregnating pitch is mixed with coke prior to melting.

2. The use as defined in Claim 1, characterized in that said member is an alkyl-aryl sulfonate.

3. The use as defined in Claim 1, characterized in that said member is selected from the class consisting of alkyl-anthracene sulfonates and alkyl-naphtalene sulfonates.

4. The use as defined in Claim 1, 2 or 3, characterized in that said member is present in an amount between 100-5000 ppm of said pitch.

5. The use as defined in Claim 1, 2 or 3, characterized in that said member is an alkyl-aryl sulfonate having an ion selected from the group consisting of sodium, potassium and ammonium.

## Patentansprüche

1. Verwendung einer aktiven Komponente mit mindestens einer Verbindung, ausgewählt unter Alkylarylsulfonsäure und Alkylarylsulfonaten, wobei die Alkylgruppe der Arylsulfonsäure oder des Arylsulfonats unter verzweigten und geradkettigen Alkylgruppen mit 1 bis 4 Kohlenstoffatomen ausgewählt wird und die Sulfonate Metallsalze, ausgewählt unter den Gruppen 1 und 2 des Periodensystems, oder Ammoniumsalze sind, in einem Verfahren zur Herstellung von Elektroden mit guter Oxidationsbestähdigkeit bei hoher Temperatur, gekennzeichnet durch Behandeln eines Bindemittels oder Imprägniermaterials für Elektroden mit einer wirkungsvollen Menge der aktiven Komponente über dem Erweichungspunkt des Pechs, jedoch bei einer Temperatur nicht über 200°C, wobei die Verbindung im geschmolzenen Zustand mit dem Pech verträglich und im Pech löslich ist, die Menge unter 1 Gew.-% des Pechs beträgt und das Pech, wenn es Imprägnierpech ist, vor dem Schmelzen mit Koks vermischt wird.

2. Verwendung nach Anspruch 1, dadurch gekennzeichnet, dass die Verbindung ein Alkylarylsulfonat ist.

3. Verwendung nach Anspruch 1, dadurch gekennzeichnet, dass die Verbindung unter Alkylanthracensulfonaten und Alkylnaphthalinsulfonaten ausgewählt wird.

4. Verwendung nach Anspruch 1, 2 oder 3, dadurch gekennzeichnet, dass die Verbindung in einer Menge von 100 bis 5000 ppm des Pechs vorhanden ist.

5. Verwendung nach Anspruch 1, 2 oder 3, dadurch gekennzeichnet, dass die Verbindung ein Alkylarylsulfat mit einem Ion, ausgewählt unter Natrium, Kalium und Ammonium, ist.

## Revendications

1. Utilisation d'un constituant actif comprenant au moins un élément choisi dans la classe constituée des acides alkyl-arylsulfoniques et des alkyl-arylsulfonates, dans laquelle le groupe alkyle de cet acide arylsulfonique ou de cet arylsulfonate est un élément choisi dans la classe constituée des éléments alkyle ramifiés et non ramifiés ayant de 1 à 4 atomes de carbone et les sulfonates sont des sels des métaux choisis dans la classe constituée des groupes 1 et 2 de la classification périodique, et de l'ammonium, dans un procédé pour préparer des électrodes ayant une bonne résistance à l'oxydation à haute température, qui comprend: le traitement d'un liant ou d'une matière d'imprégnation pour électrode avec une quantité efficace du constituant actif au-dessus du point de ramollissement du brai, mais à une température ne dépassant pas 200°C, cet élément étant compatible avec et soluble dans ce brai lorsqu'il est à l'état fondu, et cette quantité étant inférieure à 1% en poids de ce brai, et dans lequel le brai, lorsqu'il est un brai d'imprégnation, est mélangé avec du coke avant la fusion.

2. Utilisation suivant la revendication 1, caractérisée en ce que cet élément est un alkyl-arylsulfonate.

3. Utilisation suivant la revendication 1, caractérisée en ce que cet élément est choisi dans la classe constituée des alkyle anthracènesulfonates et des alkyle naphtalènesulfonates.

4. Utilisation suivant les revendications 1, 2 ou 3, caractérisée en ce que cet élément est présent dans une proportion comprise entre 100 et 5000 ppm de ce brai.

5. Utilisation suivant les revendications 1, 2 ou 3, caractérisée en ce que cet élément est un alkyl-arylsulfonate ayant un ion choisi dans le groupe constitué du sodium, du potassium et de l'ammonium.
